

July 2, 1935.

W. HEGMANN

2,006,891

# APPARATUS AND METHOD FOR PRODUCING METALLIC DUST

Filed Dec. 1, 1932

2 Sheets-Sheet 1



### Inventor

*W. Hegmann*

Witnesses  
H. Woodard

By A. Brewster & Co  
Attorneys.

July 2, 1935.

W. HEGMANN

2,006,891

APPARATUS AND METHOD FOR PRODUCING METALLIC DUST

Filed Dec. 1, 1932

2 Sheets-Sheet 2



Inventor

W. Hegmann

Witnesses  
H. Woodard

By *A. Blodgeson & Co.*  
Attorneys.

## UNITED STATES PATENT OFFICE

2,006,891

APPARATUS AND METHOD FOR PRODUCING  
METALLIC DUST

William Hegmann, Centralia, Ill.

Application December 1, 1932, Serial No. 645,306

8 Claims. (Cl. 23—139)

The invention relates to the manufacture of metallic dust by directing a blast of air against molten metal. Heretofore, the manufacture of metallic dust in this manner, has been accompanied by two drawbacks, one being the inability to produce dust sufficiently fine for a great number of purposes, and the other being the waste of compressed air (only a small percentage of that discharge serving as an actual aid in production of the dust).

My invention aims primarily to overcome the above-mentioned drawbacks, and it aims further to provide for efficient and economical oxidizing of the metallic dust if desired.

With the foregoing in view, the invention resides in the novel subject matter hereinafter described and claimed, description being accomplished by reference to the accompanying drawings.

Fig. 1 is a vertical sectional view showing one form of construction for producing metallic dust.

Fig. 2 is a vertical sectional view showing another form of construction.

Fig. 3 is a diagrammatic view showing additional apparatus used with that shown in Fig. 2, when oxidized metallic dust is to be produced.

The apparatus shown in Fig. 1 is for the production of unoxidized metallic dust. In this view, the numeral 5 denotes a suitable crucible for the molten metal and 6 has reference to an air line leading from a source of compressed air to supply the air with which to treat the molten metal. Tapped into the crucible 5 or otherwise placed in communication with the latter, is a tubular conductor 7 for the molten metal, said tubular conductor being stepped at 8 to reduce the diameter of its outer end. This outer end is formed with a small molten metal discharge opening 9 which is co-axial with the conductor 7, and the front end of said conductor is provided with a conical surface 10, through the apex of which the molten metal is discharged from the opening 9.

A sleeve or jacket 11 surrounds the conductor 7 and may be secured thereon by any preferred means, a set screw 12 being shown for illustrative purposes. The front portion of the sleeve or jacket 11, being spaced from the reduced or stepped front end of the conductor 7, provides an air chamber 13 into which the line 6 discharges, and due to the fact that the conductor 7 becomes highly heated by contact with the molten metal, the air in the chamber 13 will become pre-heated to aid materially in the production of the metallic dust. A front wall 14 is provided for the sleeve or jacket 11, said wall being secured in

place by any preferred means, a ring nut 15 being shown for this purpose. The wall 14 is formed with a frusto-conical air discharge opening 16 which is concentric with the conical surface 10 of the molten metal conductor 7 and is spaced outwardly from the latter to provide a passage 17 of annular form, the shape of said passage being such that the apparatus will discharge a hollow conical blast 18 of air directed toward its own apex, with said apex immediately in front of and axially aligned with the opening 9. The inner wall of the passage 17 extends entirely to the wall of the opening 9, and said passage and opening have their delivery ends disposed at a single transverse plane to simultaneously release the air and molten metal. The opening 9 delivers the molten metal directly into the hollow of the hollow conical air blast 18 and withdraws said molten metal from release until it can immediately impinge upon said blast. The contact of the molten metal with the air blast takes place the moment the metal leaves the metal-discharge opening and the vertex of said air blast is focused upon the stream of metal at a point in front of and co-axial with the opening 9, and the action of the compressed air on the molten metal, commutes the latter to an unusual degree of fineness. I attribute this to a large extent to the fact that there is no interval between the time the molten metal leaves the opening 9 and the time it contacts with the air blast 18, due to comparisons which I have made between the present apparatus and a somewhat analogous apparatus in which an annular blast of air is discharged around and initially parallel with the discharging stream of molten metal. When this latter arrangement is used, the air blast creates suction upon the metal discharge opening and it is this suction which induces the discharge of the molten metal, and this metal does not contact with the air blast until it has traveled quite an appreciable distance under the influence of the suction. This suction thus acts on the metal during this period of travel, as to produce the effect of spraying the molten metal into the air blast with the spray insufficiently fine to produce powder of the desired fineness when said spray is solidified by contact with the air blast. With my apparatus, the molten metal is not induced to flow by suction. In fact, the conical air blast 18 creates such a back pressure through the metal discharge opening 9 that an appreciable head of molten metal is necessary in the crucible 5, in order to overcome said back pressure and deliver the molten metal into the hollow vertex of the air blast. There is thus no

- suction-induced spraying of the molten metal and it travels no distance whatever after leaving the opening 9 before it comes in contact with the air blast 18. This air blast therefore serves as the 5 means for comminuting the molten metal and the dust produced is much finer than that possible of production when initially directing the air blast substantially parallel with the outgoing stream of molten metal. Furthermore, 10 with the present invention, there is no interval between the time the air blast leaves the passage 17 and the time said air blast comes in contact with the molten metal. The air therefore, with no chance to expand and lose part of its velocity and pressure, performs the comminution 15 more successfully than would be possible if the air were required to travel even a short distance from the passage 17, before striking the molten metal discharged through the opening 9. I, therefore, consider this bringing together of the conical air blast and the molten metal, instantaneously with the discharge of both thereof, a very important feature of the invention.
- In Fig. 2, an apparatus is shown which may 20 be used by itself for producing unoxidized metallic dust, or may be employed with the additional apparatus of Fig. 3, or some similar apparatus, to produce oxidized metallic dust. In this form of the invention, I provide a tubular conductor 25 7<sup>a</sup> for the molten metal, in the form of a hollow substantially cylindrical body which may be placed in communication with a crucible by means of a suitable conducting line 19. The front end 10<sup>a</sup> of the conductor 7<sup>a</sup> is externally 30 shaped in the same manner as the end 10 of the conductor 7 but the molten metal discharge opening 9<sup>a</sup> through the apex of this conical end, is relatively large. An appropriate jacket 11<sup>a</sup> having a compressed air inlet 6<sup>a</sup> is suitably secured 35 around the front portion of the conductor 7<sup>a</sup> and is provided with a front wall 14<sup>a</sup> co-operating with the conductor end 10<sup>a</sup> in providing an annular discharge passage 17<sup>a</sup> for discharging a hollow conical blast 18<sup>a</sup> of compressed air, which 40 blast comes in contact with the molten metal, the moment the two leave the openings 17<sup>a</sup> and 9<sup>a</sup>. An air-conducting tube 20 has its discharge end disposed centrally within the molten metal discharge opening 9<sup>a</sup>, said tube extending longitudinally 45 through the conductor 7<sup>a</sup>. Compressed air discharged through this tube into the vertex of the hollow conical blast of air, assists materially in effecting the desired comminution of the metal to an extremely fine state. Obviously, 50 the air flowing through the tube 20 will be heated by the molten metal within the conductor 7<sup>a</sup>, and the air in the chamber 13<sup>a</sup> from which the blast 18<sup>a</sup> is discharged, will be similarly heated, and all of this air-heating contributes to the best 55 results.
- By discharging fuel oil under pressure through the tube 20, the apparatus shown in Fig. 2 may be used with an apparatus such as that shown in Fig. 3, for producing oxidized metallic dust. 60
- 65 The fuel is preheated in passing through the tube 20 to facilitate the combustion necessary to produce the oxidizing. The spray of oil and metal dust is directed into a refractory lined furnace 21, where combustion of the oil takes place, and
- 70 75 the finely divided metal is readily oxidized, and then conveyed through appropriate cooling trails 22 to a suitable filtering and collecting unit 23. The filtering means 24 of this unit may well be woolen bags which allow all products of combustion to pass therethrough but retain the fine

oxidized dust which is collected in hoppers 25. Similar hoppers 26 may be employed at the lower ends of some of the trails 22, to receive relatively coarse dust.

It will be seen from the above, that the apparatus shown in Figs. 1 and 2, when used for producing unoxidized metallic dust, carry out the steps of discharging a hollow conical air blast, feeding molten metal under pressure into the hollow within said air blast, and withholding discharge of both the air blast and the molten metal until they can impinge upon each other instantaneously with their discharge. Further, with regard to the apparatus shown in Fig. 1, it will be observed that it carries out the steps of discharging a hollow conical blast of gas, and delivering molten metal only into the hollow vertex of said blast, the metal being withheld from contact with the blast until it has reached said vertex. In using the construction shown in Fig. 2, it carries out the steps of discharging a hollow conical blast of air, delivering a tubular stream of molten metal under pressure into the hollow within said air blast, withholding release of both the air blast and the molten metal until they can immediately impinge upon each other, and discharging an additional air blast along the axis of the tubular stream of molten metal.

When using the apparatus shown in Fig. 2 for the production of oxidized metallic dust, it carries out the steps of discharging a hollow conical air blast, feeding a tubular stream of molten metal under pressure into the hollow within said air blast, withholding release of the molten metal until it can immediately impinge upon the air blast, and discharging fuel into said hollow along the axis of said tubular stream of molten metal.

The apparatus shown in Fig. 1 may be used in the production of oxidized metallic dust for the reason that any metal in a finely divided state 40 is more easily oxidized when placed in a heated oxidizing atmosphere. The structure shown in Fig. 2 embodies the required provision for producing the heated oxidizing atmosphere and the air which is utilized to comminute the metal, aids 45 the combustion of the oil so that effective heating of the chamber 21 (Fig. 3) is effected. Neither the structure shown in Fig. 1 nor that disclosed in Fig. 2 will by itself actually oxidize the metallic dust, but both of these structures render the 50 comminuted metal more readily susceptible to oxidation when used with other necessary oxidizing equipment.

I claim:—

1. An apparatus for producing metallic dust, 55 comprising means for discharging a hollow conical blast of air traveling toward its own vertex, and molten metal conducting means for delivering molten metal into the hollow vertex of said blast, said blast discharging means and said 60 molten metal conducting means being related to effect contact of the air and molten metal instantaneously with the discharge of both thereof.

2. In an apparatus for producing metallic dust, 65 means for discharging a stream of molten metal under pressure, said means having a continuous-walled discharge opening for the metal, and means for discharging a hollow conical blast of air against the metal stream, said air discharge 70 means having an annular air discharge opening whose inner wall extends entirely to the wall of said molten metal discharge opening, both walls of said annular air discharge opening being positioned and shaped to focus the vertex of the 75

- air blast at a point in front of and co-axial with said metal discharge opening, said metal discharge opening and said air blast discharge opening both having their discharge ends disposed at a single transverse plane to effect contact of the air blast and molten metal instantaneously with the discharge of both thereof.
3. An apparatus for producing metal dust comprising a tubular conductor for molten metal, said conductor being externally stepped to reduce its outer end, the outer extremity of said outer end being externally conical and having a small molten metal discharge opening at the apex of the core, a separate sleeve surrounding said conductor, said sleeve fitting snugly around the larger end of said conductor and being radially spaced from the reduced end thereof, a front wall closing the outer end of said sleeve, said front wall having a frusto-conical opening spaced radially from said conical end of said conductor and co-acting therewith in forming an annular passage for discharging a conical blast of compressed air into the molten metal stream discharged through said molten metal discharge opening, said discharge opening and said annular passage having their discharge ends disposed at a single transverse plane, and a compressed air inlet into the space between said reduced conductor end and said sleeve.
4. A structure as specified in claim 2; together with a continuous-walled fluid discharge passage having its delivery end within and concentric with said metal discharge opening.
5. In a method of the class described, the steps of discharging a hollow conical air blast
- traveling toward its own apex, feeding molten metal under pressure into the hollow within said air blast, and effecting contact of the molten metal and the air blast instantaneously with the discharge of both thereof.
6. In a process for producing metallic dust, the steps discharging a hollow conical blast of air traveling toward its own apex, delivering molten metal only into the hollow vertex of said blast, and effecting contact of the molten metal and air blast instantaneously with the discharge of both thereof.
7. In a method of producing metallic dust, the steps of discharging a hollow conical air blast traveling toward its own apex, feeding a tubular stream of molten metal under pressure into the hollow within said air blast, effecting contact of said air blast and said tubular stream of molten metal instantaneously with the discharge of both thereof, and simultaneously discharging an additional air blast into said hollow along the axis of said tubular stream of molten metal.
8. In a method of producing oxidized metallic dust, the steps of discharging a hollow conical air blast traveling toward its own apex, feeding a tubular stream of molten metal under pressure into the hollow within said air blast, effecting contact of said air blast and said tubular stream of molten metal instantaneously with the discharge of both thereof, and simultaneously discharging fuel into said hollow along the axis of said tubular stream of molten metal.

WILLIAM HEGMANN. 35